

# United States Patent

Wilhelmi

[15] 3,644,251

[45] Feb. 22, 1972

[54] **NONWOVEN FABRICS AND BINDERS  
THEREFOR**

[72] Inventor: Werner Alfred Wilhelmi, Bussum, Netherlands

[73] Assignee: Nederlandsche Bewoerd Maatschappij N.V.

[22] Filed: Apr. 8, 1969

[21] Appl. No.: 814,456

[52] U.S. CL..... 260/26, 117/140 A, 117/161 K,  
117/161 KP, 117/161 P, 117/161 UB, 117/161 UF,  
117/168, 260/24, 260/27 R, 260/27 BB

[51] Int. Cl..... C08d 9/12, C08g 17/16, D06n 3/04

[58] Field of Search..... 260/24, 26, 27, 117/140 A

[56] **References Cited**

UNITED STATES PATENTS

3,380,851 4/1968 Lindemann et al. .... 117/140

|           |         |                  |         |
|-----------|---------|------------------|---------|
| 3,419,465 | 12/1968 | Maruta .....     | 162/168 |
| 3,451,890 | 6/1969  | Stump .....      | 162/168 |
| 3,490,937 | 1/1970  | Pietsch .....    | 117/63  |
| 3,510,344 | 5/1970  | Dunderdale ..... | 117/76  |

*Primary Examiner*—Hosea E. Taylor

*Assistant Examiner*—Ronald W. Griffin

*Attorney*—Daniel J. Reardon, Saul R. Bresch, George E. Lilly  
and Evelyn Berlow

[57]

## ABSTRACT

Nonwoven fabrics that have excellent wet strength and dry strength are formed by adding to an aqueous suspension of natural and/or synthetic fibers a binder comprising (a) an anionic polymer latex and (b) a mixture of alkali metal salts of disproportionated rosin and fortified rosin, precipitating the binder on the fibers, and forming the treated fibers into a non-woven fabric.

14 Claims, No Drawings

**NONWOVEN FABRICS AND BINDERS THEREFOR**

This invention relates to nonwoven fabrics and to a method for their production. It further relates to adhesive binders that are used in the production of nonwoven fabrics.

Nonwoven fabrics are composed of loosely assembled webs of natural and/or synthetic fibers that are bound together with an adhesive binder. Two general procedures are used commercially for the production of nonwoven fabrics. In the "dry process" a web of fibers, which is formed, for example, by carding or garnetting, is impregnated with a binder, and the treated web is then dried. In the "wet process," an aqueous suspension of the fibers is formed, a binder is added to the aqueous suspension and precipitated on the fibers, and the treated fibers are formed into a mat using papermaking equipment, such as fourdriniers or Rotoformers. For many applications, the wet process of producing nonwoven fabrics is preferred over the dry process because it yields superior products and because it permits higher production rates. Because the fibers are deposited with three-dimensional random orientation, the products of the wet process have equal strength in all directions, whereas in the products of the dry process the fibers are ordinarily oriented parallel to the machine direction. In addition, the products of the wet process are stronger and more uniform throughout the fiber mat because the binder is applied uniformly to the fibers in the aqueous suspension.

A number of polymers have been proposed as binding agents for nonwoven fabrics. Among them are acrylic resins, styrene-butadiene, copolymers, polyurethane, polyesters, polyamides, polyvinyl acetate, polyvinyl chloride, chlorinated polypropylene, and synthetic and natural rubber. None of these binders has given entirely satisfactory results when used in the production of nonwoven fabrics by the wet process because the polymers are not adequately retained on the fibers and the products produced do not have the desired combination of properties, and particularly good wet strength and dry strength.

In accordance with this invention, it has been found that nonwoven fabrics that are characterized by excellent tensile strength, softness, flexibility, and other valuable properties result when the binder used in the aforementioned wet process comprises a polymer latex and a mixture of alkali metal salts of disproportionated rosin and fortified rosin. The properties of nonwoven fabrics prepared using the novel binders of this invention are in many ways superior to those of nonwoven fabrics prepared from binders that do not contain the mixture of modified rosin salts. Of particular importance is the higher tensile strength of the products of this invention.

Nonwoven fabrics are prepared in accordance with the process of this invention by forming a dilute aqueous suspension of fibers, adding to the suspension and precipitating on the fibers in the suspension a binder comprising a polymer and a mixture of alkali metal salts of disproportionated rosin and fortified rosin, forming the treated fibers into a nonwoven fabric, and drying the fabric.

Any of the natural fibers and synthetic fibers that are commonly used in the production of nonwoven fabrics can be used in the practice of this invention. These include, for example, cotton, hemp, rayon, regenerated cellulose, cellulose acetate, wool, jute, polyamides, polyesters, acrylics, polyolefins, polyvinyl chloride, and polyurethane as well as mixtures of these fibers. It is generally preferred that the length of the fibers used in the present process be in the range of about 5 to 30 mm.

The binders that are applied to the fibers comprise an anionic polymer latex and about 3 to 50 percent, and preferably 5 to 20 percent, based on the weight of polymer in said latex, of a mixture of alkali metal salts of disproportionated rosin and fortified rosin.

The polymer latexes that may be present in the novel binders include solutions, emulsions, and dispersions of such polymers as acrylic resins, styrene-butadiene copolymers, polyurethanes, polyesters, polyamides, chlorinated polypropylene, polyvinyl acetate, and mixtures thereof. Par-

ticularly satisfactory results have been obtained using a binder in which the anionic polymer latex is an emulsion of an acrylic resin. As used herein, the term "acrylic resin" includes a number of polymers prepared by the polymerization of an acrylic monomer, such as acrylic acid, methacrylic acid, ethyl acrylate, butyl acrylate, cyclohexyl acrylate, methyl methacrylate, butyl methacrylate, 2-ethylhexyl methacrylate, acrylonitrile, methacrylonitrile acrylamide, methacrylamide, N-methylolacrylamide, N-methylolmethacrylamide, and mixtures thereof alone or in combination with such comonomers as styrene, ethylene, propylene, butadiene, isoprene, chloroprene, itaconic acid and the like. Illustrative of the acrylic resins that are preferred for use in the novel binders are the following: poly (ethyl acrylate), poly (methyl methacrylate), poly (2-ethylhexyl acrylate), polyacrylonitrile, ethyl acrylate/methacrylic acid, butyl acrylate/acrylic acid, acrylonitrile/butadiene/styrene, acrylonitrile/acrylic acid/butadiene, butyl acrylate/butyl methacrylate/acrylic acid, methyl acrylate/acrylic acid/ethylene, butyl acrylate/N-methylolmethacrylamide/vinyl acrylate, ethyl acrylate/styrene/N-methylolacrylamide/divinylbenzene, acrylonitrile/butadiene, 2-ethylhexyl acrylate/acrylonitrile/itaconic acid, and acrylonitrile/methacrylic acid/butadiene.

The anionic polymer latexes may be formed by any suitable and convenient procedure. For example, they may be formed by preparing a polymerization mixture containing water, the appropriate monomers, a free-radical polymerization initiator, and an anionic emulsifying agent and heating the mixture at a temperature in the range of about 80° to 90° C. until the polymerization has been completed. Among the anionic emulsifying agents that can be used are glycerol monostearate, sodium oleate, potassium oleate, triethanolamine oleate, sodium lauryl sulfate, and alkyl aryl sulfonates. The anionic polymer latex generally contains about 10 to 70 percent by weight of the polymer. Latexes having a solids content of about 35 to 50 percent are ordinarily preferred.

In addition to the aforementioned components, the anionic polymer latex may also contain defoaming agents, wetting agents, dyes, fillers, and the like in the amounts usually used for these purposes.

The mixture of rosin salts that is present in the binders of this invention contains about 50 to 90 percent by weight of an alkali metal salt of disproportionated rosin and about 10 to 50 percent by weight of an alkali metal salt of fortified rosin. Binders that have excellent retention characteristics and that form the most satisfactory products contain a mixture of salts that consists of 70 to 80 percent by weight of sodium, potassium, and/or lithium salts of disproportionated rosin and 20 to 30 percent by weight of sodium, potassium, and/or lithium salts of fortified rosin, with optimum results being obtained when the mixture contains about 75 percent by weight of the potassium salt of disproportionated rosin and about 25 percent by weight of the potassium salt of fortified rosin.

The mixture of modified rosin salts may be prepared, for example, by mixing together the appropriate amounts of the individual salts. Alternatively, a mixture of disproportionated rosin and fortified rosin may be saponified by heating it with an aqueous solution of an alkali metal hydroxide, oxide, or carbonate, and preferably with an aqueous solution of potassium hydroxide. If desired, the alkali metal salt of disproportionated rosin and the alkali metal salt of fortified rosin may be added separately to the polymer latex to form the binding agents of this invention. The mixture of modified rosin salts or the individual salts are preferably added as a dilute aqueous dispersion or solution to the other components to form the binders.

The disproportionated rosin from which the alkali metal salt is formed may be prepared by known procedures from wood rosin, gum rosin, or tall oil rosin. For example, the rosin may be disproportionated by heating it at a temperature between 150° and 300° C. in the presence of a catalyst, such as palladium, platinum, nickel, iodine, sulfur, or sulfur dioxide. A suitable method for the disproportionation of rosin is described in U.S. Pat. No. 2,138,183.

The fortified rosin that is used in the practice of this invention may be prepared by heating rosin with about 1.9 to about 7.5 percent of its weight of formaldehyde or a formaldehyde-yielding compound, such as paraformaldehyde or trioxane, at a temperature between 125° and 200° C. in the presence of an acid catalyst, such as sulfuric acid or p-toluenesulfonic acid, to form formaldehyde-modified rosin. The formaldehyde-modified rosin is then heated at a temperature between 160° and 220° C., and preferably between 175° and 195° C., with about 4 to 12 percent, and preferably 5 to 7 percent, by weight of an alpha, beta-unsaturated carboxylic acid component, such as maleic, fumaric, erotonic, acrylic, methacrylic, itaconic, citraconic, andaconitic acids, their anhydrides, their esters, and mixtures thereof. Alternatively, the fortified rosin can be prepared by heating rosin with the appropriate amounts of an alpha, beta-unsaturated carboxylic acid component at a temperature between 160° and 220° C. without the formaldehyde treatment until a product having the desired acid number is obtained.

Nonwoven fabrics may be prepared from fibers and the novel binders by procedures that are well known in the art. The procedure is usually carried out in a papermaking machine or fiber mat machine that comprises a headbox, de-watering boxes, a suction box, and a wire on which the fabric is formed. The headbox is equipped with an agitator that keeps the fibers in suspension and that assists in the uniform distribution of the binder and fixing agent throughout the suspension.

In a preferred embodiment of the invention the fibers are added to water in the headbox to form an aqueous suspension containing about 0.005 to 0.10 percent by weight of the fiber. To this suspension is added a dilute aqueous solution of a cationic fixing agent, such as a cationic ureaformaldehyde resin, melamine-formaldehyde resin, dicyandiamide-formaldehyde resin, guanidine-formaldehyde resin, polyethylenimine, polyamide, or polyamidoamine resin. The amount of fixing agent that is used is not critical provided that it is sufficient to precipitate substantially all of the binder that is subsequently added. To the resulting suspension is slowly added a dilute aqueous solution of the binder or, if desired, separate dilute solutions of the anionic polymer and the salts of modified rosin. In most cases about 50 to 200 parts by weight of the binder is added per 100 parts by weight of dry fibers, with about 60 to 110 parts by weight of binder per 100 parts by weight of dry fibers preferred. A few minutes after the addition of the binder the filtrate becomes clear, which indicates that substantially all of the binder has been fixed on the fibers. The amount of water added with the binder is such that the suspension contains about 0.05 to 1.0 gram of treated fibers per liter. The treated fibers are formed into a sheet and dried. The resulting nonwoven fabrics are soft and flexible and have excellent tensile strength.

In another preferred embodiment of the invention, the dilute aqueous binder solution is added to the aqueous suspension of fibers prior to the addition of the cationic fixing agent.

The invention is further illustrated by the examples that follow. In these examples all parts and percentages are parts by weight and percentages by weight.

#### EXAMPLE 1

A mixture of modified rosin salts was prepared by the following procedure:

- A. Fortified rosin was prepared by heating a mixture of 90 parts of rosin, 9 parts of maleic anhydride, and 1.7 parts of paraformaldehyde at 175°-180° C. for 90 minutes.
- B. Disproportionated rosin was prepared by heating rosin at 250°-310° C. for about 5 hours in the presence of a 5 percent palladium-on-carbon catalyst.
- C. To a mixture of 345 parts of disproportionated rosin and 115 parts of fortified rosin was added 70 parts of potassium hydroxide. The resulting mixture contained 75 percent by weight of the potassium salt of disproportionated rosin and 25 percent by weight of the potassium salt of fortified rosin.

#### EXAMPLE 2

- A. A suspension of 100 parts (dry weight) of polyester fibers in about 500,000 parts of water was prepared. To this suspension which was vigorously agitated was added a dilute aqueous solution that contained 4.8 parts of a cationic urea-formaldehyde resin. To the resulting suspension was slowly added a dilute aqueous dispersion that contained (a) 60 parts of an anionic polymer latex that was an anionic emulsion that contained 50 percent of poly (ethyl acrylate) and (b) 3 parts of the product of Example 1. About 10 minutes after the dispersion had been added, the filtrate was clear. The treated fibers were formed into a sheet and dried. The resulting nonwoven fabric, which was soft and resilient, had a tensile strength of 210 kg.
- B. In a comparative experiment, the above procedure was followed except that the product of Example 1 was not added to the dispersion that contained the poly (ethyl acrylate). The resulting nonwoven fabric had a tensile strength of 40 kg.
- C. In a comparative experiment, the potassium salt of disproportionated rosin was used in place of the product of Example 1. The tensile strength of the resulting nonwoven fabric was 120 kg.

#### EXAMPLE 3

To dilute aqueous suspension containing 100 parts (dry weight) of polyamide fibers was added a dilute aqueous solution that contained 4.8 parts of a cationic urea-formaldehyde resin. To the resulting suspension was slowly added a dilute aqueous dispersion that contained (a) 100 parts of an anionic polymer latex that contained 50 percent of a polymer of 94 percent of n-butyl acrylate, 5 percent of N-methylolacrylamide, and 1 percent of vinyl acrylate and (b) 5 parts of the product of Example 1. About 10 minutes after the dispersion had been added, the filtrate was clear. The treated fibers were formed into a sheet and dried. The resulting nonwoven fabric was soft and had excellent wet strength and dry strength.

#### EXAMPLE 4

To a dilute aqueous suspension containing 100 parts (dry weight) of polyurethane fibers was added a dilute aqueous dispersion that contained (a) 80 parts of an anionic polymer latex that contained 35 percent of poly (propyl acrylate) and (b) 2 parts of the product of Example 1. To the resulting slurry was added a dilute aqueous solution containing 5 parts of a cationic polyamidoamine resin. The treated fibers were formed into a sheet and dried. The resulting nonwoven fabric was soft and resilient, and it had excellent wet strength and dry strength.

The terms and expressions that have been used are as terms of description and not of limitation. There is no intention in the use of such terms and expressions of excluding any equivalents of the features shown and described or portions thereof. It is recognized that various modifications are possible within the scope of the invention claimed.

What is claimed is:

1. A nonwoven fabric comprising a web of fibers bonded with a binder that comprises (a) a polymer latex, said latex containing about 10 to 70 percent by weight of a polymer selected from the group consisting of acrylic resins, styrene-butadiene polymers, polyurethanes, polyesters, polyamides, chlorinated polypropylenes, polyvinyl acetate, and mixtures thereof and (b) 3 to 50 percent, based on the weight of polymer in said latex, of a mixture of rosin salts, said mixture containing about 50 to 90 percent by weight of an alkali metal salt of disproportionated rosin and about 10 to 50 percent by weight of an alkali metal salt of fortified rosin, said fortified rosin being the product obtained by heating rosin or formaldehyde-modified rosin and about 4 to 12 percent by weight of an alpha, beta-unsaturated carboxylic acid component at a temperature in the range of 160° to 220° C.

2. A nonwoven fabric as set forth in claim 1 wherein polymer in the latex is an acrylic resin.

3. A nonwoven fabric as set forth in claim 1 wherein the binder contains 5 to 20 percent, based on the weight of polymer in the binder, of said mixture of rosin salts.

4. A nonwoven fabric as set forth in claim 1 wherein the mixture of rosin salts contains 70 to 80 percent by weight of an alkali metal salt of disproportionated rosin and 20 to 30 percent by weight of an alkali metal salt of fortified rosin.

5. A nonwoven fabric as set forth in claim 1 wherein the mixture of rosin salts contains about 75 percent by weight of the potassium salt of disproportionated rosin and about 25 percent by weight of the potassium salt of fortified rosin.

6. A binder for nonwoven fabrics comprising (a) a polymer latex, said latex containing about 10 to 70 percent by weight of a polymer selected from the group consisting of acrylic resins, styrene-butadiene polymers, polyurethanes, polyesters, polyamides, chlorinated polypropylenes, polyvinyl acetate, and mixtures thereof and (b) 3 to 50 percent, based on the weight of polymer in said latex, of a mixture of rosin salts, said mixture containing about 50 to 90 percent by weight of an alkali metal salt of disproportionated rosin and about 10 to 50 percent by weight of an alkali metal salt of fortified rosin, said fortified rosin being the product obtained by heating rosin or formaldehyde-modified rosin and about 4 to 12 percent by weight of an alpha, beta-unsaturated carboxylic acid component at a temperature in the range of 160° to 220° C.

7. A binder for nonwoven fibers as set forth in claim 6 wherein the polymer latex is an anionic emulsion containing 35 to 50 percent by weight of an acrylic resin.

8. A binder for nonwoven fabrics as set forth in claim 6 wherein the polymer latex is an anionic emulsion containing about 50 percent by weight of poly (ethyl acrylate).

9. A binder for nonwoven fabrics as set forth in claim 6 that contains 5 to 20 percent, based on the weight of polymer in the binder, of said mixture of rosin salts.

10. A binder for nonwoven fabrics as set forth in claim 6 wherein the mixture of rosin salts contains 70 to 80 percent by weight of the potassium salt of disproportionated rosin and 20 to 30 percent by weight of the potassium salt of fortified rosin.

11. In the process for the production of nonwoven fabrics wherein a dilute aqueous suspension of fibers is formed, a binder comprising a polymer is added to said suspension, the polymer is precipitated onto said fibers, and the treated fibers are formed into a sheet and dried, the improvement that comprises incorporating in said binder 3 to 50 percent, based on the weight of polymer in said binder, of a mixture of rosin salts containing about 50 to 90 percent by weight of an alkali metal salt of disproportionated rosin and about 10 to 50 percent by weight of an alkali metal salt of fortified rosin, said fortified rosin being the product obtained by heating rosin or formaldehyde-modified rosin and about 4 to 12 percent by weight of an alpha, beta-unsaturated carboxylic acid component at a temperature in the range of 160° to 220° C.

12. The process of claim 11 wherein 5 to 20 percent, based on the weight of polymer in the binder, of said mixture of rosin salts is incorporated into the binder.

13. The process of claim 11 wherein the mixture of rosin salts contains 70 to 80 percent by weight of an alkali metal salt of disproportionated rosin and 20 to 30 percent by weight of an alkali metal salt of fortified rosin.

14. The process of claim 11 wherein the mixture of rosin salts contains about 75 percent by weight of the potassium salt of disproportionated rosin and about 25 percent by weight of the potassium salt of fortified rosin.

\* \* \* \* \*

35

40

45

50

55

60

65

70

75